

## UNITED STATES PATENT OFFICE

1,968,223

## PROCESS OF TREATING PAPER PULP

Gotthard Rosen, Paris, France

No Drawing. Application November 23, 1932,  
Serial No. 644,135. In France November 25,  
1931

13 Claims. (Cl. 92—9)

It is known that paper pulp made from wood through the soda or sulphate processes cannot be bleached, or at least cannot be bleached as easily as bisulphite paper pulp. Besides, if said pulps 5 are bleached the resulting product is more or less yellowish. Up to the present time, the kraft pulp, which contains a considerable percentage of matters that are not baked or are only half baked, could not possibly be bleached.

10 In order to render that pulp capable of being bleached, it is therefore necessary to purify it so as to diminish as far as possible the percentage of lignin, resin, incrustating bodies, etc., before subjecting the pulp to the bleaching treatment.

15 It is known that a treatment or even a supplementary heating of the pulp with a rather concentrated soda lye is capable of efficaciously purifying the pulp. That treatment or that heating operation is however very expensive and they 20 have the further disadvantage that the fibers are attacked, with a resulting considerable decrease of the yield and also a lower mechanical resistance. It has also been proposed to let the pulp remain for a certain time in tanks or vats 25 containing lime-milk, which is also capable of purifying the cellulose. However, such a method necessitates a very long treatment.

The object of my invention is to provide a 30 process of treating paper pulp through which it is possible to transform the soda pulp or sulphate pulp into a pulp that can be easily bleached. The process according to my invention consists essentially in subjecting the pulp successively to washing in a very diluted alkaline lye, washing 35 in a very hot solution of an alkaline-earth base and chlorine water or soluble chlorides, and an acid treatment. The process according to my invention is very little expensive and can be applied for industrial purposes without necessitating any 40 expensive supplementary plant.

After the residual lye has been eliminated from the pulp and after the ordinary washing, the pulp is subjected to a second washing in a very diluted alkaline lye (up to 1% NaOH, or NaOH mixed 45 with Na<sub>2</sub>CO<sub>3</sub>). That washing treatment may be performed at a temperature of about 80–90° C. In some cases the temperature may be as high as 110° C. if the treatment is performed under a pressure of about 1 kilogram per square centi- 50 meter. After removing the lye, which may be utilized two or three times, the mass is first rinsed in ordinary water, and the pulp is subjected to a third washing in a hot solution of an alkaline earth base and chlorine water or soluble chlorides 55 (for instance up to 0.4% CaO and 0.4% NaCl).

A circulation of the liquid during the two washing operations above mentioned can eventually be provided.

After removing the solution used for the third washing, the pulp is subjected to the ordinary 60 treatments until it reaches the refining piles.

A small quantity of the lime and of the salt is absorbed by the mass and remains therein during these ordinary treatments while the purifying of the cellulose is being carried on.

If the pulp is sufficiently well cooked, the second washing, that is the washing with an alkaline lye, can be dispensed with. In that case, the third washing, that is the washing with a solution of an alkaline earth and of a salt, may be prolonged. 70

When the pulp has reached the piles, the mass is treated with a dilute solution of sulphuric acid (about 3 kilograms of sulphuric per 100 kilograms of dry pulp). When the pulp has assumed a homogeneous colour, a solution of sodium chloride 75 is added (about 2 or 3 kilograms per 100 kilograms of dry pulp).

When that treatment, which lasts for a period of time ranging between half an hour and one hour, the pulp is washed with ordinary water. The 80 pulp is then ready to be washed through any of the known processes.

Through this treatment with sulphuric acid, the remainder of the lime is eliminated. At the same time a large proportion of the remaining 85 hemi-cellulose is dissolved in the acid and is removed. The pulp then assumes a lighter colour.

The soda pulp or the sulphate pulp that has been thus treated can then be bleached as easily 90 as bisulphite pulp.

In the case of the pulp being intended for the viscose artificial silk industry, for the nitro-cellulose industry, etc., it is highly important that the pulp should contain a minimum of ashes. Now, through the treatment of the pulp with sulphuric acid, there is formed calcium sulphate, which is not soluble, and consequently cannot be eliminated through washing with water. The calcium sulphate is then precipitated onto the fibers and therefore causes an increase of the 100 percentage of ashes in the pulp. In order to diminish that percentage, it is therefore preferable to make use of an acid other than sulphuric acid for the last step of the process according to my invention. It is advantageous to choose an acid 105 which gives with alkaline earth bases salts that are soluble in water, for instance hydrochloric acid, or even sulphurous acid in dilute solution.

In another mode of carrying out my invention, the pulp may be subjected first to one of the 110

washing treatments above referred to (very dilute alkaline solution, or hot solution of an alkaline earth base and of chlorine water or soluble chlorides), at a relatively low temperature, which 5 may however be as high as 70-80° C., then to an acid treatment, for instance in sulphuric acid of very low concentration. The pulp thus treated is then subjected to a preliminary bleaching step with, for instance, from 1 to 2% of active chlorine. 10 Said chlorine may be supplied by a solution of calcium chloride  $\text{CaOCl}_2$  or calcium hypochlorite (eau de Javel).

After that preliminary bleaching operation, the pulp is subjected to the other washing operation 15 (hot solution of an alkaline earth base and chlorine water or soluble chlorides, or very dilute alkaline solution, as the case may be) and then to an acid treatment, for instance with hydrochloric acid that is not very much concentrated.

19 After washing in ordinary water, the subsequent bleaching operation is performed in the known manner.

The process according to my invention is particularly well adapted for sulphate pulp or soda pulp, but it will readily be understood that it may 5 be of very high interest for other paper pulps, for instance for bisulphite pulp.

What I claim is:

1. A method of treating paper pulp and particularly soda pulp and sulphate pulp, which comprises subjecting the pulp to a washing with a dilute solution of lye, to a washing with a hot solution of an alkaline earth base and of a chlorine containing water-soluble material of the group 35 comprising chlorine and soluble chlorides, and to an acid treatment, whereby the pulp thus treated can be easily bleached.

2. A method of treating paper pulp and particularly soda pulp and sulphate pulp, which 40 comprises subjecting the pulp to a washing with a dilute alkaline lye, to a washing with a hot solution of an alkaline earth base and of a soluble chloride, and to an acid treatment, whereby the pulp thus treated can be easily bleached.

3. A process of treating paper pulp and particularly soda pulp or sulphate pulp, which comprises subjecting the pulp to an ordinary washing, to a washing with a hot solution of an alkaline earth base in a liquid containing chlorine, and to 45 an acid treatment, whereby the pulp thus treated can be easily bleached.

4. A process of treating paper pulp and particularly soda pulp or sulphate pulp, which comprises subjecting the pulp to an ordinary washing, to a washing with a dilute alkaline lye, to a washing with a hot solution of an alkaline earth base in a liquid containing chlorine, and to an acid treatment, whereby the pulp thus treated can be easily bleached.

5. A process of treating paper pulp and particularly soda pulp or sulphate pulp, which comprises subjecting the pulp to an ordinary washing, to a washing with a dilute alkaline lye, to a washing with a hot solution of an alkaline earth base in chlorine water, and to an acid treatment, whereby the pulp thus treated can be easily bleached.

6. A process of treating paper pulp and particularly soda pulp and sulphate pulp, which comprises subjecting the pulp to an ordinary washing, then to a washing with a dilute alkaline lye, to a washing with a hot solution of an alkaline earth base and a soluble chloride, and to an acid treatment, whereby the pulp thus treated can be easily bleached.

7. A process of treating paper pulp and particularly soda pulp and sulphate pulp, which comprises subjecting the pulp to an ordinary washing, then to a washing with a dilute alkaline lye, to a washing with a hot solution of an alkaline earth base in chlorine water, and to the action of sulphuric acid, whereby the pulp thus treated can be easily bleached.

8. A process of treating paper pulp and particularly soda pulp and sulphate pulp, which comprises subjecting the pulp to an ordinary washing, then to a washing with a dilute alkaline lye, to a washing with a hot solution of an alkaline earth base in chlorine water, and to the action of hydrochloric acid, whereby the pulp thus treated can be easily bleached.

9. A process of treating paper pulp and particularly soda pulp and sulphate pulp, which comprises subjecting the pulp to an ordinary washing, then to a washing with a dilute alkaline lye, to a washing with a hot solution of an alkaline earth base in chlorine water, and to the action of sulphurous acid, whereby the pulp thus treated can be easily bleached.

10. A process of treating paper pulp and particularly soda pulp and sulphate pulp, which comprises, subjecting the pulp to an ordinary washing, then to a washing with a dilute alkaline lye, to a washing with a hot solution of an alkaline earth base and a soluble chloride, and to the action of sulphuric acid, whereby the pulp thus treated can be easily bleached.

11. A process of treating paper pulp and particularly soda pulp and sulphate pulp, which comprises, subjecting the pulp to an ordinary washing, to a washing with a dilute alkaline lye, to a washing with a hot solution of an alkaline earth base and of a soluble chloride, and to the action of hydrochloric acid, whereby the pulp thus treated can be easily bleached.

12. A process of treating paper pulp and particularly soda pulp and sulphate pulp, which comprises, subjecting the pulp to an ordinary washing, to a washing with a dilute alkaline lye, to a washing with a hot solution of an alkaline earth base and of a soluble chloride, and to the action of sulphurous acid, whereby the pulp thus treated can be easily bleached.

13. A process of treating paper pulp and particularly soda pulp and sulphate pulp, which comprises, subjecting the pulp to a washing with a dilute alkaline lye at a temperature of less than 80°, subjecting to an acid treatment, and then to a preliminary treatment by means of chlorine, washing with a hot solution of an alkaline earth base in a liquid containing chlorine, and treating by an acid.

GOTTHARD ROSEN.

80

85

90

95

100

105

110

115

120

125

130

135

140